

## UNITED STATES PATENT OFFICE

HOWARD SCOTT, OF WILKINSBURG, PENNSYLVANIA, ASSIGNOR TO WESTINGHOUSE ELECTRIC &amp; MANUFACTURING COMPANY, A CORPORATION OF PENNSYLVANIA

## COMPOSITE CONDUCTOR

No Drawing.

Application filed February 8, 1930. Serial No. 427,060.

My invention relates to composite conductors having such a coefficient of expansion that they may be effectively sealed into glass, and more particularly to a composite wire having an inner core composed of an alloy containing iron, nickel and cobalt.

An object of my invention is to provide a composite wire having an outer sheath or jacket of copper and a core composed of an alloy having a lower coefficient of expansion than iron-nickel alloys.

Another object of my invention is to provide an effective seal between a vitreous envelope, such as glass, and a metal conductor composed of an outer sheath or jacket composed of copper and an inner core containing iron, nickel and cobalt, the sectional area of the copper and the inner core being maintained in such proportions that the mean coefficient of expansion of the metal conductor will range from 5 to  $7 \times 10^{-6}$  per degree centigrade from zero to 250° C.

Another object of my invention is to provide a composite metal conductor that has a sufficiently low coefficient of expansion to permit its being sealed into hard glass having a coefficient of expansion ranging from 3 to  $5 \times 10^{-6}$  per degree centigrade.

A further object of my invention is to provide a method of effecting a seal between a copper-coated conductor and glass which comprises forming a glass beading on the conductor, inserting the beaded conductor through an aperture in the glass, fusing the glass thereto, and maintaining the fused joint at the lowest temperature at which strains are effectively eliminated for a period of from 1 to 24 hours before cooling to normal temperatures.

Composite wires having an inner core composed of an iron-nickel alloy and an outer sheath or jacket of copper have heretofore been employed for conducting electrical energy into vitreous envelopes, such as glass. In utilizing such conductors, it has been necessary to maintain the cross-sectional area of the copper and the inner core in such proportions that the coefficient of expansion of the conductor and the glass will be substantially the same. In order to provide a

conductor having such a coefficient of expansion, the cross-sectional area of the core must be about 85% of the cross-sectional area of the composite conductor.

Nickel steel, however, has a resistivity of about  $70 \times 10^{-6}$  ohms per centimeter cube, and since the copper occupies only a relatively small proportion of the total cross-sectional area, the resistivity of the composite wire is approximately  $11 \times 10^{-6}$  ohms per centimeter cube.

I have made the discovery that when an iron-nickel-cobalt alloy or an iron-nickel-cobalt steel is employed as the core in a composite wire having an outer jacket of copper, the proportion of the cross-sectional area of the copper may be increased and a composite conductor formed which may be effectively sealed into an envelope composed of soft glass, or the coefficient of expansion of the composite wire may be reduced to such an extent that it may be effectively sealed into hard glass.

For example, the coefficient of expansion of a core composed of nickel steel is about  $5.5 \times 10^{-6}$  per degree centigrade, while the coefficient of expansion of an iron-nickel-cobalt alloy containing 32% nickel and 10% cobalt is approximately  $3.5 \times 10^{-6}$  per degree centigrade. An iron-nickel-cobalt alloy also has the additional advantage that it has a lower resistivity than nickel steel. The mean coefficient of expansion of composite wires that are employed for sealing into soft glass is approximately  $8 \times 10^{-6}$  per degree centigrade. When a core composed of an iron-cobalt-nickel alloy having the composition specified is employed in place of nickel steel, the cross-sectional area of the copper may, therefore, be doubled and the cross-sectional area of the core correspondingly reduced without increasing the coefficient of expansion of the composite wire. Since the resistivity of copper, however, is considerably less than the core material, the resistivity of the composite wire will be reduced to about  $5 \times 10^{-6}$  ohms per centimeter cube.

Composite wires have heretofore been employed only for making seals in soft glass, such as lead glass, which has a coefficient of

expansion of approximately  $9 \times 10^{-6}$  per degree centigrade. Their use has been limited in this respect because a sufficiently low expansion could not be obtained over the required 5 temperature range with a composite wire having a nickel-steel core and an outer jacket of copper which could be sealed into hard glass and still have a moderate resistivity. When an iron-nickel cobalt alloy, however, is 10 employed as a core, a composite wire can be produced which is capable of being sealed into a glass or vitreous envelope having a coefficient of expansion of  $6 \times 10^{-6}$  per degree centigrade. For example, a composite wire 15 having a core composed of an alloy containing 20% to 30% nickel and 18% to 28% cobalt and an outer sheath or jacket of copper occupying 10% to 30% of the total cross-sectional area, will have substantially 20 the same coefficient of expansion as hard glass, such as that known in the art as borosilicate thermometer glass, and will have a resistivity of about  $8 \times 10^{-6}$  ohms per centimeter cube.

While an alloy having specific proportions 25 of iron, nickel and cobalt has been mentioned, it will be understood that the proportions of these ingredients may be varied widely, depending upon the cross-sectional area of the copper and the composition of 30 the glass into which the conductor is to be sealed. A small proportion of manganese is also preferably added to such alloys to increase their forgeability and the usual impurities associated with the ingredients may 35 be present, although the amount of carbon should preferably be maintained below .5%. Alloys containing 45% to 66% iron, 20% to 34% nickel, 4% to 28% cobalt and 0 to 1% manganese have been found satisfactory, the 40 proportion of the ingredients in the alloy depending upon the expansivity desired and the cross-sectional area of the copper. An alloy containing 25% to 34% nickel, 4% to 17% cobalt, 0 to 1% manganese and the re- 45 mainder iron and minor impurities has been found suitable for sealing into soft glass when the cross-sectional area of the copper is maintained between 10% and 40%. By reducing the cross-sectional area of the cop- 50 per to approximately 5% to 20%, the coefficient of expansion of the composite conductor can be reduced to 3 to  $5 \times 10^{-6}$  per degree centigrade and can, therefore, be effectively sealed through an envelope composed of hard 55 glass, such as that which is commercially known as Nonex.

The values given in the foregoing examples do not represent the lowest resistivities but only those which may be obtained by conventional methods. It is possible to produce a core having a lower resistivity by certain refinements, such as by reducing the manganese content or by increasing the ratio of cobalt to nickel. By such methods, it is possible to 60 obtain a copper-jacketed core which is ca-

pable of being successfully sealed into hard glass having a coefficient of expansion of approximately  $4 \times 10^{-6}$  per degree centigrade which will have a fairly high conductivity.

My improved composite wire may be effectively sealed into the glass envelope in any desired manner. I prefer, however, to first form a glass beading on the conductor which may have the same composition as the glass envelope or a composition having a coefficient of expansion intermediate the coefficient of expansion of the glass and that of the composite wire. The beaded glass may then be inserted through an aperture in the glass envelope, and the contacting glass of the envelope and the beading are fused and pressed thoroughly in contact with each other.

In forming an effective seal between glass and a metal which is "wetted" by glass, such as copper, it is only necessary to have the mean coefficient of expansion of the metal the same as that of the glass from atmospheric temperatures to that at which strains in either the glass or metal are rapidly released. The softening temperature of copper is below that of glass. Consequently, with a copper-jacketed conductor, it is only necessary that the mean coefficient of expansion of the composite wire shall be equal to that of glass up to the softening temperature of copper. In certain constructions, and especially where good conductivity is desired, I have found that if, after sealing the conductor into the glass, the temperature is maintained at the lowest point at which strains are effectively eliminated for a period of one to twenty-four hours, the expansivity of the composite wire may be substantially reduced. For copper-jacketed wires having an iron-nickel-cobalt core, I have found that the strains may be eliminated by maintaining the seal at a temperature of from 200° C. to 300° C. for one to twenty-four hours. When such a process is followed, the cross-sectional area of the copper-jacket may be increased and the conductivity correspondingly improved. The above process also enables the seal to be cooled to normal temperature at a comparatively fast rate.

While I have described my invention in considerable detail and have given numerous examples, it will be understood that my invention is not limited to the specific details set forth in the foregoing examples which should be construed as illustrative and not by way of limitation and in view of the numerous modifications which may be effected therein without departing from the spirit of my invention, it is desired that only such limitations shall be imposed as are indicated in the appended claims.

I claim as my invention:

1. A composite wire comprising a core composed of an iron base alloy containing 25% to 34% nickel, 4% to 17% cobalt and a small

70

75

80

90

95

100

105

110

115

120

125

130

percentage but not more than 1% of manganese, and an outer jacket formed of copper, the cross sectional area of the copper being maintained at 10% to 40% of the cross sectional area of the wire.

5 2. A composite wire comprising a core composed of an iron base alloy containing 25% to 34% nickel, 4% to 17% cobalt and a small percentage but not more than 1% of manganese; and an outer jacket of copper, the cross sectional area of the copper being maintained between 5% to 20% of the cross sectional area of the wire, the coefficient of expansion of the composite conductor varying from 3 to  $5 \times 10^{-6}$  per degree centigrade.

10 15 In testimony whereof, I have hereunto subscribed my name this 6th day of February, 1930.

HOWARD SCOTT.

20

25

30

35

40

45

50

55

60

65